

## UNITED STATES PATENT OFFICE

FRANK A. FAHRENWALD, OF CHICAGO, ILLINOIS, ASSIGNOR TO AMERICAN MANGANESE STEEL COMPANY, OF CHICAGO, ILLINOIS, A CORPORATION OF MAINE

METHOD OF INCREASING THE STRENGTH, TOUGHNESS, AND DUCTILITY OF MANGANESE STEEL

No Drawing.

Application filed March 26, 1928. Serial No. 264,972.

My invention relates to the heat treatment of articles made of manganese steel and is based upon the discovery that certain deficiencies in the manganese steel can be overcome by heat treating in the novel manner hereinafter described.

While manganese steel has long been noted for its toughness, shock resistance, and wear resistance it has failed to satisfactorily meet certain industrial requirements because of its low elastic strength and general initial softness. Many attempts have been made in the past, both by myself and by other investigators, to raise the physical strength, and particularly the yield point of manganese steel by changing its composition or by adding other alloying elements thereto. None of these have proved successful, however, and up to the time of my present invention it has generally been considered impossible to effect substantial improvements in this direction. I have discovered, however, that if manganese steel be heated in an atmosphere of hydrocarbon gas without carburizing effect upon the metal of the articles, for instance in the heating step preliminary to the usual quenching operation, the resulting castings are from a fifth to a third stronger and considerably tougher and more ductile than manganese articles heat-treated by the usual methods. In the ordinary method of heat treating manganese steel as practiced heretofore, the castings or other articles were heated in a fuel fired or electrically heated chamber to a temperature around 1,800° F. (or around 980° C.) and maintained at that temperature for a sufficient time to insure uniformity and then quenched in water.

Instead of heating manganese steel as previously in the ordinary products of combustion or in the oxidizing atmosphere of the electric furnace, my process subjects manganese steel articles to radiant heat in a spacious chamber containing free, unoxidized hydrocarbon gas; the chamber being heated preferably, either externally by fuel-firing or internally by means of electrical resistance elements mounted within the chamber. The manganese steel articles so treated, when subsequently quenched, possess character-

istics never heretofore found in manganese steel castings processed by any other method. In the case of small cast manganese steel chain, for instance, treated by this process, the breaking strength is approximately 17,000 pounds, whereas the same chain treated by previous methods would only sustain 13,000 pounds, and in the case of test bars heat-treated before machining to standard dimensions, the difference between gas treated and ordinary treated castings, determined for me by a reputable commercial testing establishment and which is typical of the relative value of the new manganese steel as against manganese steel produced by the old standard method, is represented by the following figures:

Physical properties of manganese steel

|                   | Heated in ordinary furnace | Heated in hydro-carbon atmosphere | 70 |
|-------------------|----------------------------|-----------------------------------|----|
| Yield point       | 48,230                     | 60,140                            | 75 |
| Ultimate strength | 116,930                    | 130,480                           |    |
| Elongation        | 34%                        | 42%                               |    |
| Reduction of area | 25%                        | 42%                               |    |

I make no attempt to explain the chemical or other reactions which may combine to produce this remarkable improvement, and simply claim the process and the products as such. In my new process practically any low sulphur hydrocarbon gas, such as natural or artificial illuminating gas, or vapors of alcohol, or gasoline, or volatile distillation products of coal may be employed; and the treatment temperature should be above about 1650° F. or above 900° C.

As a typical procedure and the best way now known to me of carrying out the invention, introduce the manganese steel castings, unboxed and fully exposed, into the heating chamber of an electric resistance furnace, and at or before the time that the castings begin to show color, introduce ordinary illuminating gas into the same chamber with freedom of convection and in quantity sufficient to quickly consume the oxygen in the chamber and cause the atmosphere to assume a smoky reducing condition. Continue or repeat the

introduction of the gas in a small flow or quantity sufficient to maintain this character of atmosphere to the end of the heating step, and until the discharge door is about 8 to be opened and the castings raked out.

This process is not to be confused with the process of case hardening ordinary types of steels, wherein only the surface and not the interior of the steel is made to absorb carbon, 10 and where the absorption of carbon is of such a high degree that when quenched after heating, an extremely hard surface is produced. In my process for the treatment of manganese steel in an atmosphere containing free hydro- 15 carbon gas, there is no carburizing of the metals of the articles and of the surface of the articles, in fact, the surface is somewhat softer than results from treatment by ordinary means, as practiced heretofore; and the ef- 20 fects of the hydrocarbon environment occur while the metal is at temperature appropriate for quenching, and are followed by quenching, which circumstances may have their influence upon the surprising results obtained 25 from the procedure.

I claim:

1. The process of heat treating manganese steel articles, which comprises the steps of subjecting said articles to a temperature 30 above about 1650° F. (above about 900° C.) and maintaining around said articles, at least while they are at such temperature, a non- carburizing environment containing hydro- 35 carbon gas and without carburizing the metal of the articles, and then quenching said articles.

2. The improvement in the art of heat- 40 treating manganese steel articles, which consists in carrying out the critical portion of the heating step which is preliminary to quenching, while the manganese steel articles are exposed to a freely convective hydrocarbon containing reducing atmosphere but without carburizing the metal of the articles, 45 and by subjection to a heat source which is independent of said atmosphere, and then quenching the articles.

3. The improvement in the art of heat 50 treating articles of manganese steel, which consists in bringing such articles up to the quenching temperature of said treatment and, at least while the articles are at said temper- 55 ature, exposing them directly to a substan- tially unignited, non-carburizing environ- ment containing a readily oxidizable gas without carburizing the metal of the articles, and then quenching the articles.

4. In the art of heat treatment of articles 60 of manganese steel, the improvement which consists in maintaining around the articles from about the time the articles attain crit- 65 ical temperature to the time of attaining quenching temperature and until the articles are withdrawn for quenching, a non-carbu- 70 rizing atmosphere containing free hydrocar-

bon gas, and thereby completing the heating step without carburizing the metal of the ar- 75 ticles.

Signed at Chicago Heights, Illinois, this 70 6th day of March, 1928.

FRANK A. FAHRENWALD.

75

80

85

90

95

100

105

110

115

120

125

130

**CERTIFICATE OF CORRECTION.**

**Patent No. 1,834,206.**

**Granted December 1, 1931, to**

**FRANK A. FAHRENWALD.**

**It is hereby certified that error appears in the printed specification of the above numbered patent requiring correction as follows: Page 2, line 16, after "and" insert no hardening; and that the said Letters Patent should be read with this correction therein that the same may conform to the record of the case in the Patent Office.**

**Signed and sealed this 16th day of February, A. D. 1932.**

**(Seal)**

**M. J. Moore,  
Acting Commissioner of Patents.**